

## UNITED STATES PATENT OFFICE

2,046,296

## ACOUSTICAL PAINT

Carlisle K. Roos, Wheaton, James S. Offutt, Chicago, and Herman A. Scholz, Oak Park, Ill., assignors to United States Gypsum Co., Chicago, Ill., a corporation of Illinois

No Drawing. Application May 31, 1930,  
Serial No. 458,926

12 Claims. (Cl. 134-46) 106 - 79

This invention relates to plastic compositions, and has reference more particularly to plastic compositions for application to the walls and ceilings of buildings for the purpose of correcting the acoustical properties in said building.

In correcting the acoustical properties of rooms and buildings it is customary to apply an acoustical plaster, or other surface, to the ceilings or walls of the room, in a comparatively thick layer for absorbing the sound waves and preventing echoes in the room. Fiber boards and hair felt have been used for this purpose but they are unsightly in appearance and give little or no decorative effect. After a period of time, these acoustical materials become soiled through use and rather unsightly, so that it is desirable to apply a thin layer of an acoustical paint over the acoustical material to give a fresh and clean surface and improve the appearance of the room. However, it is important that this acoustical paint applied to the acoustical plaster does not appreciably reduce the sound absorbing qualities of the acoustical material. It is also sometimes desirable to apply an acoustical paint in a rather thick, sound absorbing layer over a room surface which in itself is not sound absorbing, or over an old and soiled coating of acoustical paint. The decorative effect may also be produced by texturing our acoustical paint.

An object of this invention, therefore, is to provide a composition which is suitable for application over acoustical plaster, boards, tiles or mats for the purpose of improving the appearance and decorative effect of same.

Another object of the invention is to provide an acoustical composition which may be applied to building surfaces, for the purposes of absorbing sound waves; also to improve acoustical surfacing materials in other respects hereinafter specified and claimed.

Our improved composition is primarily intended for brush application to the surfaces of buildings for the purpose of absorbing impinging sound waves. It preferably contains a substantial amount of fibrous materials, and in order to secure proper brush application, we have found it necessary to provide special pre-treatment of the fibers in order to secure a uniform dispersion of same, as well as other qualities. This pre-treatment of the fibrous material consists essentially in coating the fibers with a binder by mixing the fibrous material with the solution containing the binding material, drying, grinding and grading the product. While one pretreatment may be sufficient in certain cases, we have found that two or more pretreatments are desirable, and we shall designate these pretreatments as pretreatment "M" and pretreatment "N". The pretreatments very materially improve the plasticity and brushability of our acoustical product.

Pretreatment "M" is prepared by adding a mixture of the following:

| Parts by weight                              |      |   |
|----------------------------------------------|------|---|
| Mineral wool                                 | 66.4 | 5 |
| Asbestos No. 7 BM                            | 3.5  |   |
| Pine sawdust (white pine, graded)            | 5.8  |   |
| Cottonwood fibers (screened to remove fines) | 5.3  |   |

|                                 |      |
|---------------------------------|------|
| to a solution of the following: | 10   |
| Processed wheat or corn paste   | 11.8 |
| Gum arabic                      | 5.3  |
| Karaya gum                      | 2.1  |
| Water                           | 23.2 |

The wetted mass is placed on screens and dried, then ground through a Prater mill or other pulverizing machine and screened so that all passes an 8 mesh screen.

Pretreatment "N" is prepared by adding a mixture of the following:

| Parts by weight                   |       |    |
|-----------------------------------|-------|----|
| Mineral wool                      | 45.2  |    |
| Asbestos No. 7 BM                 | 2.6   |    |
| Pine sawdust (white pine, graded) | 4.2   | 25 |
| to the following binder solution: |       |    |
| Casein                            | 32.0  |    |
| Water                             | 141.0 |    |
| Ca(OH) <sub>2</sub>               | 6.4   |    |
| Silicate of soda                  | 22.4  | 30 |

This wetted mass is spread on a screen, dried, ground through a Prater mill, and then screened so that all passes a 16 mesh screen.

Pretreatment "M" is a means of incorporating fibrous fillers, which have been wetted with an adhesive mixture. This aids in the dispersion of the fillers without greatly decreasing the fiber length of the mineral wool and cottonwood fibers, and without it the material is heavy and dense. The processed wheat or corn paste is a partially dextrinized starch. Corn or other farinaceous pastes may be used with varying success.

Pretreatment "N" contributes greatly to the porosity when used in conjunction with the other ingredients in the formula, and prevents the formation of a skin on the surface of the finished and dried acoustical paint which would reduce the porosity and sound absorbing qualities. An excess of pretreatment "N" darkens the color of the final composition and increases the number of surface cracks. It is our belief that the sodium lime caseinate precipitated on the surfaces of the fibers by the interaction of the ingredients in the pretreatment "N", swells in the wet mix, and in drying contracts, leaving open and interconnecting pores which aid the sound absorbing qualities of the composition. The sodium silicate preferred has a Na<sub>2</sub>O:SiO<sub>2</sub> ratio of 1:2.84 having 60

11 per cent  $\text{Na}_2\text{O}$  and 31.2 per cent  $\text{SiO}_2$  and a due to the increase in the percentage of pumice gravity of 47°  $\text{Bé}$ .

This pretreatment of the fibers may be accomplished in a number of different ways as long as the fibers are coated with the binding material before mixing with the main part of the composition, and only the preferred form of accomplishing these pretreatments is given below. The pretreated fibrous material may also be mixed with the other ingredients in the composition in a number of different ways, and two characteristic formulas will be given.

Formula No. 1 consists of the following ingredients:

|                                                                               | Percent |
|-------------------------------------------------------------------------------|---------|
| 15 Pumice (passing 20 mesh, retained on 48 mesh)                              | 13.0    |
| Marble (passing 20 mesh, retained on 48 mesh)                                 | 26.7    |
| 20 Cold water glue                                                            | 2.4     |
| Aluminum sulphate ( $\text{Al}_2(\text{SO}_4)_3 \cdot 18\text{H}_2\text{O}$ ) | 1.3     |
| Wheat paste                                                                   | 2.4     |
| Gum Karaya                                                                    | 1.01    |
| 25 Lithopone                                                                  | 16.0    |
| Pretreatment "M" (Precoated fibrous material)                                 | 21.0    |
| Pretreatment "N" (Precoated fibrous material)                                 | 16.0    |
| 30 Tribromophenol                                                             | 0.2     |
| Oil of sassafras, 4-5 drops per pound of composition.                         |         |

In this formula No. 1, the pumice and the marble act as an aggregate. Pumice gives bulk and porosity, although a larger amount of pumice than 13 per cent produces marked short-working characteristic in the final composition. The marble gives weight, color, and aids texturing properties besides making a small contribution to the porosity.

The glue gives a stickiness very desirable for brush application. Glue gives a great portion of the final strength and an excess of glue reduces the porosity. Bone glue has given us the best results. The alum acts as a preservative for the wheat paste and affects the viscosity of the glue. The wheat paste modifies the tenacious nature of the glue, increasing the consistency and contributing to the final strength and hardness. We believe furthermore it helps brushing characteristics and plasticity. The gum Karaya greatly increases the consistency and final porosity. It lightens the wet material and while an excess helps the porosity, it injures the application. The lithopone helps the color and brushing, giving a plasticity and gel characteristic very desirable for brush application. Its use must be controlled since an excess reduces porosity to a marked degree. The tribromophenol acts as a preservative and mold preventative. The oil of sassafras is used to mask the objectionable phenol odor of the tribromophenol.

In formula No. 2 an increase in the pumice and marble gives better porosity and lower initial cost, but there is some sacrificing of desirable working characteristics and hardness of the final formula. Oxalic acid and paraformaldehyde act as insolubilizing agents on the glue. The paraformaldehyde may be added at the job if desired to prevent any undesired reactions in the dry mixture. Sodium phosphate increases the viscosity of the glue, and gives a better body to the formula, but is not essential thereto. Other materials have been varied somewhat in proportion,

Formula No. 2 is as follows:

|                                                                               | Per-cent |
|-------------------------------------------------------------------------------|----------|
| Pumice (passing 30 mesh, retained on 48 mesh)                                 | 5        |
| Marble (passing 30 mesh, retained on 48 mesh)                                 | 16.7     |
| Cold water glue                                                               | 33.4     |
| Aluminum sulphate ( $\text{Al}_2(\text{SO}_4)_3 \cdot 18\text{H}_2\text{O}$ ) | 1.1      |
| Wheat paste                                                                   | 10       |
| Lithopone                                                                     | 2.0      |
| Pretreatment "M" (Precoated fibrous material)                                 | 12.5     |
| Pretreatment "N" (Precoated fibrous material)                                 | 16.7     |
| Oxalic acid                                                                   | 13.3     |
| Paraformaldehyde                                                              | .1       |
| Karaya gum                                                                    | 2        |
| Dibasic sodium phosphate                                                      | .83      |
|                                                                               | 1.2      |
|                                                                               | 20       |

Various materials may be substituted for those in our formulas Nos. 1 and 2, with varying success. Instead of the pumice and marble, we may use crushed, burned clay, pyrophyllite, silica, or other crushed, or graded inert materials. Instead of cold water glue, casein, blood albumen, or other binding or adhesive materials may be used.

It is thought that carbon dioxide gas is formed by the action of alum on the marble. Potassium or sodium carbonate or whiting may be added as equivalent gas forming agents to react with the alum. This generated carbon dioxide not only improves the porosity of the dried paint, but also aids materially in preventing the formation of a surface crust which would reduce the sound absorbing efficiency of the paint. Instead of the wheat paste, corn paste, tapioca or other farinaceous pastes may be used. The gum Karaya has the property of forming a thick solution with 50 to 75 parts by weight of water, and when this water dries out, it gives the resulting dried composition a porosity where the space was previously occupied by water. Gum tragacanth and Irish moss may be substituted for the gum Karaya. Instead of the lithopone, other white pigments may be used such as zinc oxide, titanium oxide pigments and white lead pigments. Other preservatives may be used instead of the tribromophenol, such as phenol, cresol or beta naphthol, etc. Other aromatic substances may be used instead of oil of sassafras, such as oil of cloves, wintergreen, pine oil, etc. Wood fibers other than cottonwood may be used. In formula No. 2 tartaric and citric acid may be substituted instead of the oxalic acid, with varying degrees of success and formaldehyde, lead acetate, or sodium or potassium dichromate may be substituted for paraformaldehyde. Instead of the dibasic sodium phosphate, monosodium phosphate, magnesium chloride, sodium hydroxide or chrome alum may be substituted. We consider glue, wheat paste, gum Karaya, tribromophenol, oil of sassafras, asbestos, cottonwood fibers, sawdust, oxalic acid, paraformaldehyde and sodium phosphate as desirable but non-essential ingredients of our composition.

Our acoustical paint may be colored in any shade by the addition of a suitable color pigment. The coloring, texturing and acoustical properties and possibilities, gives to our paint a unique field of usefulness not achieved by other methods of decorating.

We would state in conclusion that while the illustrated examples constitute practical embodiments of our invention, we do not wish to limit ourselves precisely to these details, since manifestly the same may be considerably varied without departing from the spirit of the invention as defined in the appended claims.

Having thus described our invention, we claim as new and desire to secure by Letters Patent:

10 1. The step in the preparation of an acoustical composition which comprises mixing a fibrous material with a solution containing casein, water, hydrated lime, and silicate of soda, drying said fibrous mass to precipitate coating material on 15 the surface of said fibers, and pulverizing said fibrous mass.

20 2. The method of pretreating fibrous material preparatory to mixing with an acoustical composition, which comprises precipitating a coating of sodium calcium caseinate on the fibers of the fibrous material, drying the fibrous material, and pulverizing said fibrous material.

25 3. A composition of matter for acoustical absorption of sound, having substantially the following formula:

|                                                                 | Per cent |
|-----------------------------------------------------------------|----------|
| Pumice (passing 20 mesh, retained on 48 mesh)                   | 13.0     |
| Marble (passing 20 mesh, retained on 48 mesh)                   | 26.65    |
| Cold water (bone) glue                                          | 2.4      |
| Aluminum sulphate ( $Al_2(SO_4)_3 \cdot 18H_2O$ )               | 1.3      |
| Wheat paste                                                     | 2.4      |
| Gum Karaya                                                      | 1.05     |
| Lithopone                                                       | 16.0     |
| Mixed mineral and vegetable fibers coated with a dextrin binder | 21.0     |
| Mixed mineral and vegetable fibers coated with a casein binder  | 16.0     |
| 40 Tribromophenol                                               | 0.2      |
| Oil of sassafras, 4 to 5 drops per pound of composition.        |          |

45 4. The method of preparing an acoustical composition, which comprises mixing a fibrous material with a solution containing reactive agents for precipitating a water insoluble caseinate coating material on the surface of said fibers, drying and pulverizing the wetted fibrous mass to 50 form a pretreated fibrous material, and mixing said pretreated fibrous material with a granular, inert filler, binding material selected from the group consisting of farinaceous paste, glue, casein, and blood albumen, and with gas forming agents comprising carbonates and acid salts, water absorbing gum, a pigment, and a preservative agent.

55 5. The method of preparing an acoustical composition, which comprises applying a water insoluble caseinate coating material to the surface of fibers in a fibrous mass containing mixed vegetable and mineral fibers, drying and pulverizing said mass to form a pretreated fibrous material, and mixing said pretreated fibrous material with a granular filling material, a binding agent selected from the group consisting of farinaceous paste, glue, casein and blood albumen, and with gas forming agents, comprising carbonates and acid salts, and a pigment.

70 6. The step in the method of producing an acoustical composition, which comprises mixing mineral wool, asbestos, and sawdust with a solution containing a water insoluble caseinate binding agent, and drying and pulverizing the resulting mass.

7. An acoustical composition comprising 30 to 37% of a mineral and vegetable fibrous material precoated with a mixture containing a binding material selected from the group consisting of farinaceous paste, gum Arabic, casein and sodium silicate solution, 39.7 to 50.1% of an inert filler selected from the group consisting of granular pumice, marble, burned clay, pyrophyllite, and silica, gas forming agents comprising carbonates and acid salts, a water absorbent gum, 10 and a preservative.

15 8. An acoustical paint composition comprising 13.0 to 16.7% of granular pumice, 26.7 to 33.4% of granular marble, a binding agent selected from the group consisting of farinaceous paste, 15 glue, casein and blood albumen, said composition also including gas producing agents comprising carbonates and acid salts, a gum having a high water absorbing property, and pigment, and 30 to 37% of a mixed vegetable and 20 mineral fibrous material precoated with a binder selected from the group consisting of farinaceous paste, gum Arabic, casein and sodium silicate solution.

25 9. An acoustical composition comprising 39.7 to 50.1% of a granular inert material selected from the group consisting of pumice, marble, burned clay, pyrophyllite and silica, and passing a 20 mesh screen and retained on a 48 mesh screen, 30 to 37% of mixed mineral and vegetable fibrous materials precoated with a caseinate binder, a binding agent selected from the group consisting of farinaceous paste, glue, casein and blood albumen, and agents comprising carbonates and acid salts for causing a porous structure in 35 the mass of material for the absorption of impinging sound waves.

10. An acoustical composition comprising 30 to 37% of mineral and vegetable fibrous material precoated with a mixture containing an adhesive material selected from the group consisting of farinaceous paste, Karaya gum, gum Arabic, casein, and sodium silicate; 39.7 to 50.1% of an inert filler selected from the group consisting of granular pumice, marble, burned 45 clay, pyrophyllite and silica; glue; insolubilizing agents; gas forming agents comprising carbonates and acid salts; and a water absorbing gum.

11. An acoustical composition comprising 30 to 37% of mixed mineral and vegetable fibrous material precoated with a mixture containing an adhesive selected from the group consisting of farinaceous paste, Karaya gum, gum Arabic, casein, and sodium silicate; 39.7 to 50.1% of a granular inert filler material selected from the group consisting of granular pumice, marble, burned clay, pyrophyllite and silica; said mixture also containing glue, wheat paste, a gum having a high water absorbing property; gas generating 60 materials comprising carbonates and acid salts, and a preservative.

12. The step in the preparation of an acoustical composition, which comprises mixing a fibrous material with a solution of fiber coating adhesive materials selected from the group consisting of farinaceous paste, Karaya gum, gum Arabic, casein and sodium silicate; and drying and pulverizing the wetted mass to form a pretreated material suitable for use in an acoustical coating composition.